

Sept. 23, 1952

E. D. BOLINGER ET AL

2,611,172

## APPARATUS FOR TREATING YARN

Filed June 30, 1949

2 SHEETS—SHEET 1



INVENTORS  
EDGAR DARE BOLINGER  
ROBERT G. BERNER

BY  
*John Robert James*  
AGENT

Sept. 23, 1952

E. D. BOLINGER ET AL

2,611,172

## APPARATUS FOR TREATING YARN

Filed June 30, 1949

2 SHEETS--SHEET 2



**INVENTORS**  
**EDGAR DARE BOLINGER**  
**ROBERT G. BERNER**

RV

John Robert James  
AGENT

## UNITED STATES PATENT OFFICE

2,611,172

## APPARATUS FOR TREATING YARN

Edgar Dare Bolinger and Robert G. Berner, Stamford, Conn., assignors to Deering Milliken Research Trust, Greenwich, Conn., a non-profit trust of Maine

Application June 30, 1949, Serial No. 102,364

7 Claims. (Cl. 28—28)

1

This invention relates to a method and apparatus for treating yarn and, more particularly, to a method and apparatus for treating tire cord to improve the adhesive and other physical properties thereof.

In applying a liquid adhesive and other coating and impregnating compositions to tire cord, difficulty is experienced in obtaining a thin, complete and uniform coating. Moreover, the breaking strength of tire cord is reduced if the cord is stretched while wet with liquid, because the filaments are damaged, yet stretching is very difficult to avoid, because the yarn is easily elongated even under the small stress required to draw it through the treating apparatus. At the same time, the wet yarn, if allowed to do so by reducing the tension thereon, will tend to shrink, thus increasing its capacity for elongation and reducing its strength somewhat.

A high grade tire cord must have an elongation and a breaking strength within fairly narrow limits. Smooth-surfaced cords are tailored to those limits before an adhesive is put on to improve their adhesion to rubber. Therefore the adhesive must be applied without either stretching the cord or allowing it to shrink, so that the cord's elongation and breaking strength remain unchanged.

The present invention provides an improved method and means for applying fluid material to yarn or cord in the form of a solution, emulsion or dispersion, without either stretching the yarn or allowing it to shrink.

The invention also provides an improved method and means for imparting to the tire cord, during drying of the fluid material thereon, the tension necessary either to stretch the yarn or to allow it to shrink, to bring it within the desired limits of elongation and tensile strength required of high quality tire cord.

The treating apparatus of the invention comprises means for applying fluid material to the yarn, means for drying said yarn, and cooperating drive means disposed adjacent the points at which the yarn reaches and leaves the drying means for propelling treated yarn at the desired uniform speed and tension between those points.

A preferred embodiment of the invention is illustrated in the accompanying drawings, in which:

Fig. 1 is a longitudinal vertical section through an apparatus embodying the invention, showing the path of travel of the yarn being treated while in the form of a warp through the dipping tank, dryer and delivery rolls;

Fig. 2 is a top plan view of the apparatus of Fig. 1, taken along the line 2—2 and partly broken away;

2

Fig. 3 is an enlarged side elevation of the grooved guide roll under which the yarns pass while immersed in the dipping tank;

Fig. 4 is an enlarged front perspective view of the apparatus without the splash pan, showing the guide plate, dipping tank, squeeze rolls and drain pan; and

Fig. 5 is an enlarged perspective view of the rear of the apparatus, showing the delivery rolls and drive mechanism.

The apparatus shown in the drawings comprises an elevated framework 1 at the left end of which (as viewed in Fig. 1) a dipping tank 3 is positioned on crossbars 5 and 6. Also mounted on crossbar 5 are two upright plates 7 and 8, which between them support the normally stationary guide rod 9 and the guide plate 11. The guide plate 11 is provided with two parallel rows of "eyes," indicated generally at 13, each eye being adapted to receive an individual end, indicated at Y, of yarn or cord to be treated. The rod 9 serves as a guide for assembling the yarn or cord to be treated in the form of warp W after passage through the plate 11 and prior to immersion in the dipping tank 3.

The dipping tank is provided with a guide in the form of a stationary grooved roll 14, fixedly mounted in the tank adjacent the bottom thereof on the shaft 15. The ends of the shaft 15 are supported on the parallel arms 16 and 16'. These arms are fixedly mounted at their ends upon the guide rod 9 adjacent plates 7 and 8, and are adapted to be rocked with the rod by operation of the handle 17 so that the guide roll 14 may be raised to the dotted-line position shown at "A" during threading thereof. A pair of locking bars 18 and 18' are provided to hold the roll 14 in the lowered solid-line position shown in the drawing. These bars are rotatably mounted at their upper ends in the housing 20, and immovably engage the shaft 15 adjacent the arms 16 and 16'.

The dipping tank may be provided with a cover in order to hinder loss of solvent from the treating solution, emulsion or dispersion. Also, a hood 45 may be provided to carry off solvent vapors. Liquid may be circulated through the tank by means of a propeller, if desired, in order to keep the solution, emulsion or dispersion uniform. Likewise, the treating liquid may be continuously circulated from a storage reservoir and thus maintained at constant level.

The housing 20 is positioned on the crossbar 6 and in it are mounted the bearing blocks 21 and 21' and the shaft 23. The bearing blocks 21 and 21' may be moved vertically up and down in the housing 20 and in them is journaled the ends of the shaft 22 which carries the rubber roll 24. The ends of shaft 23 are journaled in the housing;

this shaft carries the stainless steel roll 25. Rolls 24 and 25 together constitute a set of squeeze rolls which are adapted to receive the coated and impregnated warp W from the dipping tank, and remove excess treating solution from opposite surfaces of the yarn. The solution pick-up is regulated by adjusting the squeeze pressure. Excess solution is returned to the tank by the drain pan 26. The splash pan 27 is supported on and covers the upper front and rear portions of the housing 20, and prevents splatter of liquid adhesive from the squeeze rolls.

Reciprocably positioned within the housing above the bearing blocks 21 and 21' are the cross plates 28 and 29. At each end of plate 28 are dependent knife edges 30 and 30', which respectively bear in grooves 31 and 31' upon the bearing blocks 21 and 21'. Upon plate 29 is mounted a lever 32 pivoted at 33, to which lever is attached a rod or piston 34 which passes through an aperture in the plate 29 and bears upon the plate 28, which in turn acts upon bearing blocks 21 and 21' through the knife edges 30 and 30' respectively. When the free end of the lever 32 is moved downwardly, the piston 34 is forced downward against plate 28, the reaction of which thrusts the plate 29 upwardly against the inside top of the housing 20, the piston acting as a pivot for the lever during this movement. Continued downward movement of the free end of the lever increases the pressure upon plate 28 and, therefore, the pressure on the bearing blocks 21 and 21'. Roll 24 is thus brought closer to the lower roll 25 to increase the squeeze pressure at the nip of the rolls. Weights 36 at the free end of the lever thus permit adjustment of the squeeze pressure between the rolls.

The housing 40 defines the dryer, and is provided with apertures 41 and 42 for ingress and egress, respectively, of the warp W being treated. The housing 40 is supported within the framework 1 upon the base crossbars 43 and 43'. The side walls 44 and 44' of the housing carry infra-red lamps, indicated generally at 46, which are closely spaced throughout the length and width of each side wall. The housing is open at top and bottom for circulation of air therethrough by convection. If desired, fans may be provided for direct circulation of air through the housing. A set of fluted rotatable guide rolls 47, 48, 49, 50, 51, 52 and 53 whose guide ends are journaled in the frame of the dryer housing are adapted to carry the treated warp W in festoons through the dryer so that the yarns are simultaneously subjected upon opposite surfaces thereof to the rays of the lamps. More guide rolls may be added, if desired, for greater holdup length for operation at higher speeds.

As the warp of yarn passes through the dryer, a large amount of heat is applied thereto by means of the infra-red lamps, which heat vaporizes most of the water or other fluid carriers contained in the emulsion or solution absorbed by the yarn. By adjusting the number of lamps in the housing, and the rate of the passage of the warp through the housing (which in turn depend upon the speed at which the yarn is traveled, and the length of the path of the yarn through the chamber), it is possible to dry the yarn to any desired moisture content. Ordinarily, the treated yarn is dried back to the moisture content of the untreated yarn, usually between 10 and 13 per cent. The rate of drying the warp may be increased by providing means for withdrawing moisture-laden air from the

upper part of the chamber and supplying dry air at the lower part of the chamber through suitable air circulation devices. It will be understood that means for providing heat other than infra-red lamps may also be employed, such as electrical heating coils; also, heated air may be employed.

The guide rolls 47 to 53, inclusive, in the dryer housing are preferably idler rolls. In the apparatus shown in the drawings, the rolls are journaled in fixed position in the dryer housing, but some or all of the bearings or axles for these rolls may be resiliently held in place or in adjustable position therein so that the length of the path of the warp through the dryer may be varied as desired. The surface of the rolls should be such that neither the yarn nor material upon it will adhere thereto. Thus, the rolls shown are fluted. The rolls may also be smooth surfaced, and either solid or hollow and adapted to receive circulating cold water to keep them at a low temperature and thus avoid adhesion. A high vapor content of the atmosphere within the dryer may help to prevent accumulation of adhesive material on the guide rollers if the guide rollers are cooled, for in this event moisture continuously condenses upon the surface of the rollers and this moisture continuously softens any adhesive material transferred from yarn surfaces to the surface of the guide roll and thus lessens adhesion of such material to the guide roller, so that transfer of adhesive material from the yarn to the guide roll is lessened. Also in such an atmosphere a mixture of liquid condensate and adhesive material on the surface of the guide roll is more easily removed by a scraper which may also be provided, if desired.

At the right end of the platform 1, as viewed in Figs. 1, 2 and 5, a pair of upright plates 55 and 56 are mounted on crossbar 10', and support the shafts 57 and 58. The ends of shaft 57 are journaled in plates 55 and 55, and at its central portion between the plates shaft 57 carries the steel delivery roll 60. Upon the end of shaft 57 adjacent plate 56 is positioned a sprocket wheel 65 which is driven by a chain 68. This chain drive may be operated by an electric motor or other driving means (not shown). Upon the opposite end of the shaft 57 is mounted gear 70, which meshes with and drives a gear 71. The gear 71 is fixedly mounted on a bushing 72 which is rotatably mounted on a stub shaft 73 which itself is fixedly mounted upon plate 55. The gear 71, in turn, meshes with and drives a gear 75 which is fixedly mounted upon the end of a shaft 58. The ends of shaft 58 are journaled in plates 55 and 56, and at its central portion between the plates the shaft carries a steel delivery roll 78. This gear arrangement serves to drive delivery rolls 60 and 78 at the same speed. Resting upon and between rolls 60 and 78, and driven by frictional contact therewith, is a steel tension roll 79.

Likewise fixedly mounted on bushing 72 is a sprocket wheel 80 which drives a chain 82. This chain drives a sprocket wheel 85 on shaft 23, and thereby drives the stainless steel roll 25 of the pair of squeeze rolls. The upper roll 24, in turn, is driven by frictional contact with the lower roll 25. Wheels 80 and 85 are of such relative diameter, that the squeeze rolls 24 and 25 are driven at the same surface speed as the driven delivery and tensioning rolls 60, 78 and 79. Also mounted upon the upright support plates 55 and 56 through

the brackets 90 and 90' is a guide plate 91, which is provided with two parallel rows of "eyes" indicated generally at 92. Each "eye" is adapted to receive an individual yarn end. Thus, the plate 90 separates the warp W' of treated yarn or cord into a shed of individual yarn ends, Y' as it emerges from the nip of the delivery rolls 60, 78 and 79. The yarn ends Y' are borne from this point to bobbins (not shown) on which they are individually wound.

In carrying out the method of the present invention and operating the apparatus, the individual ends of yarn or cord to be treated are fed from the bobbins through the eyes 13 and then assembled in the form of a warp W by passage 15 over the guide rod 9. The warp is passed into and through the dipping tank 3 under the guide roll 14 and thence upwardly from the tank between the pair of squeeze rolls 24 and 25, whence it passes through the aperture 41 into the interior 10 of the dryer housing 40 under the guide roll 41, upwardly to the top of the dryer chamber, over the guide roll 48 and thence downwardly through the dryer chamber to the bottom thereof, under the guide roll 49 and thence upwardly to the top 15 of the dryer chamber, over the guide roll 50 and downwardly to the bottom of dryer chamber, thence under the guide roll 51 and upwardly to the top of the dryer chamber, over the guide roll 52, and finally downwardly to and under the 20 guide roll 53 and out through the aperture 42 to the delivery rolls 60, 78 and 79. The warp passes under the first driven roll 78, and thence between the nip of rolls 78 and 79, over the roll 79, between the nip of the roll 79 and the second driven roll 60 and finally beneath the second driven roll 60. This set of three delivery rolls together with the squeeze rolls 24 and 25 draw the yarn through the apparatus, including the dryer chamber and dipping tank. Since both sets of rolls are driven at the same surface speed, through the common drive chain 82, the yarn is fed into the dryer as fast as it is withdrawn therefrom, and thus is subjected to a uniform tension and is neither stretched nor allowed to shrink during the drying process. Finally, the warp of treated yarn is divided into a shed by passing through the two rows of the eyes 92 and then is wound individually on bobbins (not shown).

The process of the invention has been found to be applicable to the treatment of tire cord and yarn formed of synthetic resins, cellulose derivatives, or natural fibers, and mixtures thereof, including viscose rayon, nylon, Orlon (polyacrylonitrile), Saran (polyvinylidene chloride), Terylene (condensation products of terephthalic acid and a glycol), and cotton to improve the adhesion thereof to natural and synthetic rubber.

In treating a warp of tire cord by the method of the present invention, a suitable aqueous or organic solvent solution, emulsion or dispersion is placed in the dipping tank. The treating composition may contain a wetting agent to increase its wetting of the yarn and/or an anti-foam agent to break the foam in the dipping tank and permit high-speed operation of the machine. Solutions and dispersions which have been found to be satisfactory have a solids content between 25 and 40 per cent and a viscosity of 5 and 400 cps. 70 Those commercially available include:

1. Flintkote Syntex C-634—An aqueous alkaline ammonia dispersion of casein, reclaim rubber and rubber latex.

2. Hercules Rosin Amine D in Solvesso 100—75 a pH of 11.0.

Solution of abietic acid neutralized with ammonia and dissolved in higher alkylated aromatic solvents.

3. Flintkote 11074 GP—Solution of neoprene in toluene.

4. Flintkote 11575 D Perbunan—Acrylonitrile synthetic rubber base dissolved in methylethylketone.

10 5. Esso Perbunan Durez A 6578-1—Solution containing 100 parts acrylonitrile rubber latex and 100 parts Durez 12687 (phenol formaldehyde resin) dissolved in 300 parts methylisobutylketone.

6. Naugatuck Dispersite 1740—Same as Syntex C-634.

7. Union Bay State AD-479-3 plus MDI-50—Solution of neoprene in an organic aromatic solvent plus methylene bis-(4-phenylisocyanate).

20 8. Flintkote Syntex 11110-QW-2—An aqueous alkaline ammonia dispersion of casein and rubber latex.

9. Syntex C-634 plus Syton—An aqueous alkaline ammonia dispersion of casein, reclaim rubber, rubber latex and colloidal silica.

10. Resorcinol-Formaldehyde Latex Dispersion—An aqueous rubber latex dispersion compounded with an alkaline resorcinol-formaldehyde solution.

The yarn, in passing through the dipping tank, may absorb as much as several times its weight of emulsion or solution, and it will be apparent that a very considerable amount of heat is required to evaporate this water or solvent content. A rapid output of heat is effected through the use of infra-red radiation which serves to rapidly vaporize the water absorbed by the yarn. The rapid vaporization and withdrawal of vapor-laden air from the drying chamber serves to keep the temperature of the yarn within a safe limit. 40 If, after drying has been effected, the yarn has not yet left the drying chamber, the adhesive composition coated on the yarn is subjected to the action of the infra-red lamps and is caused to be firmly bonded to the yarn. When the adhesive coating upon the yarn is of a dark color, the use of infra-red lamps is doubly advantageous, a larger portion of the energy of the infra-red rays being converted into heat as a result. The current to the lamps may be adjusted, or the lamps be wired in parallel so as to regulate the number of lamps burning at a given time, and thus regulate the heat input.

In order to obtain strong adhesion of the rubber coating to the yarn, it may be desirable to subject the dry, coated yarn to heat for a period of time after all of the moisture has been evaporated. This further heating causes additional drying and effects a firm bond between the coating material and the yarn. Usually, however, the further heating undergone by the yarn during vulcanization is sufficient for this purpose.

60 Table I lists typical data taken during a number of runs made using solutions of Syntex C-634 having varying viscosities and solids content. Each solution was placed in the dipping tank of the apparatus shown in the drawing, and a batch of viscose rayon tire cord treated therewith.

65 Table II lists typical data taken during a run treating nylon tire core using a 30% solids solution containing 95 parts water, 12.5 parts resorcinol, 26.4 parts 37% formaldehyde solution, and 31.5 parts of 10% sodium hydroxide solution. The solution had a viscosity of 24 cps. and a pH of 11.0.

Table I

| Viscose Rayon Tire Cord                                                | Bath, Percent Solids | Viscosity (cp.) | Percent Solids Pickup | Yarn Speed (yds./min.) | Squeeze Pressure (lbs.) | Dryer Temp., °F. | Av. Tensile Strength <sup>1</sup> (lbs.) |         | Av. Percent Elongation at 10 lbs. Tension <sup>1</sup> |         | Av. Percent Moisture Regain |         |
|------------------------------------------------------------------------|----------------------|-----------------|-----------------------|------------------------|-------------------------|------------------|------------------------------------------|---------|--------------------------------------------------------|---------|-----------------------------|---------|
|                                                                        |                      |                 |                       |                        |                         |                  | Untreated                                | Treated | Untreated                                              | Treated | Untreated                   | Treated |
| 2200 Denier<br>2 ply<br>Twist: (Turns/in.)<br>9.8 singles              | 37                   | 56              | 10.1                  | 25                     | 15                      | 250              | 34.7                                     | 31.7    | 1.98                                                   | 1.8     | 9.9                         | 11.2    |
| 8.6 ply                                                                |                      |                 |                       |                        |                         |                  |                                          |         |                                                        |         |                             |         |
| 1100 Denier<br>2 ply<br>Twist: (Turns/in.)<br>14.5 singles<br>11.5 ply | 33                   | 56              | 8.9                   | 25                     | 20                      | 250              | 34.7                                     | 32.3    | 1.98                                                   | 1.8     | 9.9                         | 11.4    |
| 1650 Denier<br>2 ply<br>Twist: (Turns/in.)<br>11.5 singles<br>10 ply   | 33                   | 21              | 7.4                   | 120                    | 20                      | 250-270          | 23.35                                    | 21.18   | 5.27                                                   | 4.46    | 10.76                       | 13.15   |
| 2200 Denier<br>2 ply<br>Twist: (Turns/in.)<br>10 singles               | 37                   | 73              | 6.4                   | 26                     | 25                      | 250              | 29.04                                    | 29.49   | 4.23                                                   | 2.88    | 12.09                       | 9.94    |
| 9 ply                                                                  | 37                   | 73              | 7.1                   | 26                     | 20                      | 250              | 29.01                                    | 30.06   | 4.16                                                   | 2.89    | 12.05                       | 9.87    |
| 2200 Denier<br>2 ply<br>Twist: (Turns/in.)<br>10 singles<br>9 ply      | 35                   | 23              | 8.3                   | 26                     | 25                      | 250              | 31.18                                    | 29.02   | 3.96                                                   | 2.47    | 12.10                       | 13.60   |
| 1650 Denier<br>2 ply<br>Twist: (Turns/in.)<br>11.5 singles<br>10 ply   | 37                   | 73              | 7.2                   | 35                     | 20                      | 250              | 23.20                                    | 22.52   | 5.23                                                   | 3.40    | 10.98                       | 11.66   |
| 11.5 singles<br>10.5 cable                                             | 37                   | 73              | 7.2                   | 48                     | 10                      | 250              | 13.53                                    | 11.65   | 14.21                                                  | 11.25   | 9.93                        | 11.05   |
| 10.5 cable                                                             | 35                   | 24              | 8.2                   | 48                     | 5                       | 250              | 13.50                                    | 12.43   | 13.29                                                  | 9.65    | 9.78                        | 9.43    |

<sup>1</sup> Measurements made at 55% R. H. and 70° F.<sup>2</sup> Not determined but estimated to be 250° F.

Table II

| Nylon Tire Cord                                                                        | Bath, Percent Solids | Viscosity (cp.) | Percent Solids Pickup | Yarn Speed (yds./min.) | Squeeze Pressure (lbs.) | Adhesion—lbs./in.    |         |                |         | Av. Percent Moisture Regain |         |
|----------------------------------------------------------------------------------------|----------------------|-----------------|-----------------------|------------------------|-------------------------|----------------------|---------|----------------|---------|-----------------------------|---------|
|                                                                                        |                      |                 |                       |                        |                         | Nat. Rubber to Cord— |         | Between Plies— |         |                             |         |
|                                                                                        |                      |                 |                       |                        |                         | Untreated            | Treated | Untreated      | Treated | Untreated                   | Treated |
| 210 Denier<br>4 x 2 ply<br>Twist: (Turns/in.)<br>1.0 singles<br>12.5 ply<br>10.5 cable | 30                   | 24              | 8.6                   | 75                     | 18.5                    | 2.4                  | 15.3    | 2.8            | 19.3    | 3.66                        | 6.14    |

The following is claimed:

1. An apparatus for treating yarn comprising, in combination, means for assembling a plurality of ends of yarn in sheet form, means for supplying liquid treating material to the thus assembled ends of yarn, yarn guide means associated with said last mentioned means, a housing for passage therethrough of the treated yarn ends, locking means associated with said housing for holding said guide means in yarn engaging position, a pair of squeeze rollers disposed in said housing and engageable by the yarn ends for removing excess liquid material from said assembled treated ends, drying means for drying said assembled treated yarn ends, drawing means for the yarn ends comprising a pair of spaced rolls and an idler roll supported by, and in frictional engagement with both spaced rolls, driving means for rotating one of said pair of spaced rolls, gear means coupling said pair of spaced rolls together for driving the other of said pair of spaced rolls, means for separating said sheet of dried treated yarn ends into individual ends, and means associated with said drawing means for driving the said squeeze rollers.

2. An apparatus in accordance with claim 1 in which the yarn guide means comprises a roll provided with grooves, each of which is adapted to receive an individual yarn end.

3. An apparatus in accordance with claim 1 which includes a covering means associated with said housing for preventing splatter of liquid treating material therefrom.

4. An apparatus in accordance with claim 1 which includes means for retracting the yarn guide means during threading up.

5. An apparatus in accordance with claim 1 wherein said means for removing excess liquid material from said treated yarn ends comprises a pair of squeeze rolls, one of said rolls being formed of stainless steel and the other of said rolls being formed of rubber and including a driving connection between the drawing means and said squeeze rolls for rotating the squeeze rolls in timed relation with the rotation of said spaced rolls.

6. An apparatus in accordance with claim 5 which includes means associated with said housing for regulating the pressure between said squeeze rolls.

7. Apparatus according to claim 5 wherein said driving connection drives said squeeze rolls at the same peripheral speed as that of the driven roll of the drawing means.

EDGAR DARE BOLINGER.  
ROBERT G. BERNER.

9

## REFERENCES CITED

The following references are of record in the  
file of this patent:

## UNITED STATES PATENTS

| Number     | Name          | Date          | 5         |
|------------|---------------|---------------|-----------|
| Re. 15,631 | O'Neil        | June 19, 1923 | 2,283,014 |
| 1,608,342  | Selleys       | Nov. 23, 1926 | 2,390,001 |
| 2,040,105  | Ritzert       | May 12, 1936  | 2,410,361 |
| 2,260,860  | Newton et al. | Oct. 28, 1941 | 2,419,922 |
|            |               |               | 10        |
|            |               |               | 2,420,399 |
|            |               |               | 2,438,084 |
|            |               |               | 2,469,123 |
|            |               |               | 2,565,407 |

10

| Number    | Name      | Date          |
|-----------|-----------|---------------|
| 2,283,014 | Reid      | May 12, 1942  |
| 2,390,001 | Schindler | Nov. 27, 1945 |
| 2,410,361 | Prance    | Oct. 29, 1946 |
| 2,419,922 | Tippetts  | Apr. 29, 1947 |
| 2,420,399 | New       | May 13, 1947  |
| 2,438,084 | Wood      | Mar. 16, 1948 |
| 2,469,123 | Martin    | May 3, 1949   |
| 2,565,407 | Still     | Aug. 21, 1951 |